# EUROPEAN PATENT SPECIFICATION

(11) **EP 4 249 617 B1**
(45) Date of publication and mention of the grant of the patent: **23.07.2025**
(21) Application number: 22905478.8
(22) Date of filing: 15.09.2022
(51) Int. Cl.: C22C 21/04, C22C 1/03, B22D 17/00, B22D 17/32, B22D 21/04, C22C 21/02, C22C 1/02, C22F 1/043

(54) **HIGH-STRENGTH AND HIGH-TOUGHNESS NON-HEAT-TREATABLE DIE-CASTING ALUMINIUM-SILICON ALLOY AND PREPARATION METHOD THEREFOR**
HOCHFESTE UND HOCHZÄHE NICHT WÄRMEBEHANDELBARE ALUMINIUM-SILIZIUM-DRUCKGUSSLEGIERUNG UND HERSTELLUNG VERFAHREN DAFÜR
ALLIAGE D'ALUMINIUM-SILICIUM COULÉ SOUS PRESSION À HAUTE RÉSISTANCE ET À HAUTE TÉNACITÉ, NON TRAITABLE THERMIQUEMENT, ET MÉTHODE DE PRÉPARATION POUR CET ALLIAGE

(30) Priority: 13.01.2022 CN 202210038413
(43) Date of publication of application: 27.09.2023
(73) Proprietor: Shanghai Jiao Tong University, Shanghai 200240 (CN); Fengyang LS Light Alloy Precise Forming Co., Ltd., Chuzhou City, Anhui Province (CN)
(72) Inventor: PENG, Liming, Shanghai 200240 (CN); YUAN, Lingyang, Shanghai 200240 (CN); YANG, Lei, Shanghai 200240 (CN); XIAO, Gang, Shanghai 200240 (CN); YANG, Chao, Shanghai 200240 (CN)
(74) Representative: Bayramoglu et al.
(86) International application number: PCT/CN2022/118853
(87) International publication number: WO 2023/134190

(56) References cited:
- EP-A1- 1 978 120
- CN-A- 104 294 495
- CN-A- 104 294 495
- CN-A- 104 831 129
- CN-A- 104 831 129
- CN-A- 105 316 542
- CN-A- 105 441 737
- CN-A- 108 754 256
- CN-A- 108 754 256
- CN-A- 114 411 020

## Description

TESLA uses a heat treatment-free alloy to prepare an integrated body structural member, and the main component of the used alloy is an Al7SiMgMn alloy (the publication number of the patent: US20050167012A1). The alloy is combined with high vacuum and even ultrahigh vacuum die casting to prepare parts. By adopting the technical route, a problem of part deformation caused by an original heat-treatable alloy can be alleviated. However, there are still two major problems: (1) the Si content in the alloy is low (about 7 wt.%), and the ductility of the material can be increased to 10-15%. The low Si content restricts the flowability of the non-heat-treatable alloy, which causes a risk of short filling for a large casting. (2) An existing Al7SiMgMn alloy features low strength (the typical yield strength is 110-120 MPa and the tensile strength is 180-220 MPa), so that the overall wall thickness of the large casting in structural design is great and there are more wall thickness areas. Therefore, under circumstance of not changing or slightly reducing the ductility of the material (guaranteeing that the ductility is greater than 10% to satisfy a riveting requirement of the body structural member), to improve the flowability of the material by increasing the Si content in the alloy and improving the strength of the material is of great significance to optimize a large body casting structure.

Therefore, one of the targets pursued in the die casting field is to develop a high-strength and high-toughness non-heat-treatable die-casting aluminum-silicon alloy and study its preparation and die-casting process, so as to satisfy the actual operating requirements improved day by day on a high quality high-performance aluminum alloy die casting. CN104831129A discloses a non-heat treatment self-reinforcing aluminium-silicon alloy preparation technology, which comprises the following steps: adding pure magnesium ingot, intermediate alloys AL-Si, AL-Mn, AL-Cu, and AL-Ti in a fusing aluminium liquid at temperature of 740-760 DEG C, after fusing, insulating for 30 minutes at 740 DEG C; heating the temperature of an alloy liquid to 780 DEG C, adding mixing rare earth, removing the scummings on the surface after fusing the mixing rare earth, stirring for 3-6 minutes and increasing the temperature of the alloy liquid to 770-780 DEG C, insulating and standing for 30 minutes; finally cooling the alloy liquid to 750 DEG C for refining, refining for 15 minutes, removing the slag, degassing, and finally completing the casting production. The mixing rare earth and an element Mn are used for refining Si and Cu in an aluminium alloy material according to strict mol fraction ratio.

### SUMMARY

The objective of the present invention is to, under the background of the prior art, provide a high-strength and high-toughness non-heat-treatable die-casting aluminum-silicon alloy and a preparation method therefor. In the premise of guaranteeing good casting performance of the alloy, a non-heat-treatable casting features excellent comprehensive mechanical properties so as to satisfy the performance requirement on the body structural member, particularly a large thin-walled body structural member.

To achieve the objective, it is found in a long-term aluminum die casting alloy study that the Si content in the die-casting aluminum-silicon alloy significantly affects the casting performance, the strength and the plasticity of the alloy. Under normal circumstances, with the increase of the Si content, the strength of the alloy is increased, the flowability thereof is increased, and the plasticity thereof is reduced. Although the element Sr can play a role of modification refinement on eutectic Si in the alloy, the plasticity thereof still shows a reducing trend along with increase of the Si content. Therefore, 10% of plasticity is hardly achieved. The present invention mainly aims to solve the problem that the plasticity of the Al-Si alloy is reduced under a die-casting condition in a case where the Si content is increased. With increase of the Si content in the alloy, the content of the eutectic Si in structures is increased, and the size and shape of the eutectic Si are also changed therewith, which becomes a key factor that affects the plasticity of the alloy. To overcome reduction of the plasticity of the material due to increase of the Si content in the alloy, the present invention creatively introduces the element V to refine an eutectic Si phase, so as to obtain a fine eutectic Si structure. In addition, it is found by a plenty of experimental verifications in early stage that rare earth elements such as La, Er and Ce can be compounded with element V to further refine the eutectic Si structures in the alloy, so that the size and shape of the eutectic Si change. Due to compound addition of V+RE, fine eutectic Si particles are generated in an as-cast structure, thereby guaranteeing that a die-casting aluminum alloy material with great Si content still has high plasticity. On the one hand, by adding the high content of Si, the alloy features excellent strength and flowability. On the other hand, due to compound addition of V+RE, the eutectic Si is retained in a fine and dispersed state, so that the plasticity of the alloy is improved. Furthermore, in the premise of guaranteeing excellent casting performance, the present invention can greatly improve the mechanical performance of the die-casting aluminum-silicon alloy and obtain comprehensive mechanical properties of high strength and high toughness taking strength and shaping into consideration.

Accordingly, the objective of the present invention is realized by the following technical solution:
The present invention provides a high-strength and high-toughness non-heat-treatable die-casting aluminum-silicon alloy, including the following components in percentage by weight: 8.0-10.0% of Si, 0.1-0.5% of Mg, 0.5-0.8% of Mn, 0.05-0.5% of Cu, 0.05-0.2% of Ti, 0.01-0.05% of Sr, 0.01-0.1% of V, 0.01-0.15% of RE, less than 0.2% of Fe, less than or equal to 0.4% of other impurities, and a balance of Al.

The RE is one or more of elements La, Ce and Er.

The present invention further relates to a method for preparing a high-strength and high-toughness non-heat-treatable die-casting aluminum-silicon alloy, including the following steps:
S1: drying: pre-heating prepared raw materials: of pure Al, pure Si, pure Mg, an Al-Mn intermediate alloy, an Al-Ti intermediate alloy, an Al-Cu intermediate alloy, an Al-RE intermediate alloy, and an Al-V intermediate alloy for a drying treatment; and
S2: smelting: adding the Al-Ti intermediate alloy, the Al-Cu intermediate alloy, the Al-Mn intermediate alloy, the Al-V intermediate alloy, and the pure Si after melting the pure Al by a preliminary heating to obtain a first resulting alloy melt, and performing a cooling on the first resulting alloy melt after melting the pure Si, the Al-Ti intermediate alloy, the Al-Cu intermediate alloy, the Al-Mn intermediate alloy, the Al-V intermediate alloy to obtain a second resulting alloy melt; pressing the pure Mg into a bottom of the second resulting alloy melt for melting to obtain a third resulting alloy melt, and performing a secondary heating on the third resulting alloy melt for a refinement of the third resulting alloy melt after completely melting the pure Mg to obtain a fourth resulting alloy melt; and then pressing the Al-RE intermediate alloy into a bottom of the fourth resulting alloy melt for melting to obtain a fifth resulting alloy melt, and leaving the fifth resulting alloy melt still after completely melting the fifth resulting alloy melt to obtain the high-strength and high-toughness non-heat-treatable die-casting aluminum-silicon alloy.

As an embodiment of the present invention, preferably, a pre-heating temperature in S1 is 190-210°C.

As an embodiment of the present invention, preferably, a preliminary heating temperature in S2 is 750-760°C.

As an embodiment of the present invention, preferably, a cooling temperature in S2 is 680-700°C.

As an embodiment of the present invention, preferably, a secondary heating temperature in S2 is 720-730°C.

As an embodiment of the present invention, preferably, the refinement in S2 specifically includes: introducing a nitrogen with a refining agent powder into the third resulting alloy melt by using a rotary blowing device for an injection refining to obtain a first refined melt, performing a deslagging treatment and a degassing treatment on the first refined melt to obtain a second refined melt, then leaving the second refined melt still for 10-15 min, and completing a slagging-off treatment on the second refined melt to obtain the fourth resulting alloy melt.

As an embodiment of the present invention, preferably, process parameters for the rotary blowing device are as follows: a degassing revolution is 300-350 r/min; a degassing time is 5-10 min, a pressure of a gas source during the degassing treatment is 0.35±0.05 MPa, and a gas flow is 0.2-0.8 sccm.

As an embodiment of the present invention, preferably, the refining agent powder includes one of magnesium chloride and calcium chloride.

Compared with the prior art, the present invention has the following beneficial effects:
1. The high-strength and high-toughness non-heat-treatable die-casting aluminum-silicon alloy prepared in the present invention has important industrial application value. Under a die-casting condition, the die-casting aluminum-silicon alloy obtains excellent performance: the yield strength is 120-160 Mpa, the tensile strength is 260-320 Mpa and the ductility is 10-15% (for the AlSi10MnMg alloy, the as-cast tensile strength is 200-220 MPa, and the ductility is 5-8%). The alloy can realize good die-casting performance, which greatly satisfies the application requirement on the large thin-walled body structural member in the automobile industry.
2. Under an as cast condition, the alloy has excellent performance: the yield strength is 120-160 MPa, the tensile strength is 260-320 MPa and the ductility is 10-15%. Compared with existing heat treatable alloys, heat treatment steps for parts can be reduced, so that the percent of pass of the casting is improved and the cost of the casting is lowered.

### BRIEF DESCRIPTION OF THE DRAWINGS

By reading and referring to detailed description made by the following drawings to non-restrictive embodiments, other features, purposes and advantages of the present invention will become more obvious.

FIG. 1 shows observation schematic diagrams of SEM structures of castings in examples and comparative examples, wherein a represents the observation schematic diagram of the SEM structure of the casting A1, b represents the observation schematic diagram of the SEM structure of the casting A2, c represents the observation schematic diagram of the SEM structure of the casting A3, d represents the observation schematic diagram of the SEM structure of the casting A4, e represents the observation schematic diagram of the SEM structure of the casting A5, f represents the observation schematic diagram of the SEM structure of the casting A6, g represents the observation schematic diagram of the SEM structure of the casting A7, h represents the observation schematic diagram of the SEM structure of the casting A8, i represents the observation schematic diagram of the SEM structure of the casting A9, j represents the observation schematic diagram of the SEM structure of the casting A10, k represents the observation schematic diagram of the SEM structure of the casting A11 and l represents the observation schematic diagram of the SEM structure of the casting A12.

### DETAILED DESCRIPTION OF THE EMBODIMENTS

A high-strength and high-toughness non-heat-treatable die-casting aluminum-silicon alloy and a preparation method therefor provided by the present invention are further described below in combination with examples, so that those skilled in the art can easily understand advantages and features of the present invention, which is not used to limit the application scope of the present invention.

### Example 1

The embodiment of the present invention provide a high-strength and high-toughness non-heat-treatable die-casting aluminum-silicon alloy, including the following components in percentage by weight: 8.0% of Si, 0.25% of Mg, 0.6% of Mn, 0.15% of Ti, 0.15% of Cu, 0.02% of V, 0.025% of Sr, 0.12% of Fe, 0.3% of other impurities and the balance of Al.

Preparation and die-casting processes for the high-strength and high-toughness non-heat-treatable die-casting aluminum-silicon alloy of the embodiment include the following steps:
1) drying: prepared raw materials: pure Al, pure Si, pure Mg, an Al-10Mn intermediate alloy, an Al-10Ti intermediate alloy, an Al-50Cu intermediate alloy, and an Al-5V intermediate alloy were pre-heated to 200°C for drying treatment; and
2) smelting: a furnace was heated to 755°C to melt the pure aluminum, then the Al-10Ti, Al-50Cu, Al-10Mn, Al-5V and pure Si alloys were added into the furnace, the furnace was cooled to 690°C after the intermediate alloys were melted, the pure Mg was pressed into a bottom area of a crucible by using a bell jar for melting, and then the pure Mg was stirred for 5 min. Then a melt was heated to 720°C, nitrogen at a pressure of 0.4 MPa was introduced into the melt, a refining agent powder accounting for 0.4% of total weight of the melt was brought in, and nitrogen was introduced with a gas flow of 0.5 at 300r/min for 10 min to deslag and degas. Then the melt was left still for 12 min, slagging-off treatment was completed, and a blast furnace component analytical test was performed. High pressure casting was performed at 690°C after the test passed. An injections peed was 3 m/s, a casting pressure was 80 MPa, a ratio of a release agent was 1: 100, and a die temperature was 230°C. The die used in a production process was a die-casting test bar die, and an obtained casting was labeled as A1.

### Example 2

The embodiment of the present invention provide a high-strength and high-toughness non-heat-treatable die-casting aluminum-silicon alloy, including the following components in percentage by weight: 8.0% of Si, 0.25% of Mg, 0.6% of Mn, 0.15% of Ti, 0.15% of Cu, 0.05% of Er, 0.025% of Sr, 0.12% of Fe, 0.3% of other impurities and the balance of Al.

Preparation and die-casting processes for the high-strength and high-toughness non-heat-treatable die-casting aluminum-silicon alloy of the embodiment include the following steps:
1) drying: prepared raw materials: pure aluminum, pure Si, pure Mg, an Al-10Mn intermediate alloy, an Al-10Ti intermediate alloy, an Al-50Cu intermediate alloy, and an Al-10Er intermediate alloy were pre-heated to 200°C for drying treatment; and
2) smelting: a furnace was heated to 755°C to melt the pure aluminum, then the Al-10Ti, Al-50Cu, Al-10Mn and pure Si alloys were added into the furnace, the furnace was cooled to 690°C after the intermediate alloys were melted, the pure Mg was pressed into a bottom area of a crucible by using a bell jar for melting, and then the pure Mg was stirred for 5 min. Then a melt was heated to 720°C, nitrogen at a pressure of 0.4 MPa was introduced into the melt, a refining agent powder accounting for 0.4% of total weight of the melt was brought in, and nitrogen was introduced with a gas flow of 0.5 at 300r/min for 10 min to deslag and degas. Then the melt was left still for 12 min, and slagging-off treatment was completed; after refining was completed, the Al-10Er intermediate alloy was pressed into the bottom area of the crucible by using the bell jar for melting, and then the Al-10Er intermediate alloy was stirred for 5 min till the Al-10Er intermediate alloy was completely melted, and then the melt was left still for 12 min, and a blast furnace component analytical test was performed. High pressure casting was performed at 690°C after the test passed. An injections peed was 3 m/s, a casting pressure was 80 MPa, a ratio of a release agent was 1: 100, and a die temperature was 230°C. The die used in a production process was a die-casting test bar die, and an obtained casting was labeled as A2.

### Example 3

The embodiment of the present invention provide a high-strength and high-toughness non-heat-treatable die-casting aluminum-silicon alloy, including the following components in percentage by weight:8.0% of Si, 0.25% of Mg, 0.6% of Mn, 0.15% of Ti,0.15% of Cu, 0.02% of V, 0.05% of Er, 0.025% of Sr, 0.12% of Fe, 0.3% of other impurities and the balance of Al.

Preparation and die-casting processes for the high-strength and high-toughness non-heat-treatable die-casting aluminum-silicon alloy of the embodiment include the following steps:
1) drying: prepared raw materials: pure aluminum, pure Si, pure Mg, an Al-10Mn intermediate alloy, an Al-10Ti intermediate alloy, an Al-50Cu intermediate alloy, an Al-10Er intermediate alloy and an Al-5V intermediate alloy were pre-heated to 200°C for drying treatment; and
2) smelting: a furnace was heated to 755°C to melt the pure aluminum, then the Al-10Ti, Al-50Cu, Al-10Mn, Al-5V and pure Si alloys were added into the furnace, the furnace was cooled to 690°C after the intermediate alloys were melted, the pure Mg was pressed into a bottom area of a crucible by using a bell jar for melting, and then a melt was stirred for 5 min. Then the melt was heated to 720°C, nitrogen at a pressure of 0.4 MPa was introduced into the melt, a refining agent powder accounting for 0.4% of total weight of the melt was brought in, and nitrogen was introduced with a gas flow of 0.5 at 300r/min for 10 min to deslag and degas. Then the melt was left still for 12 min, and slagging-off treatment was completed; after refining was completed, the Al-10Er intermediate alloy was pressed into the bottom area of the crucible by using the bell jar for melting, and then the Al-10Er intermediate alloy was stirred for 5 min till the intermediate alloy was completely melted, and then the melt was left still for 12 min, and a blast furnace component analytical test was performed. High pressure casting was performed at 690°C after the test passed. An injections peed was 3 m/s, a casting pressure was 80 MPa, a ratio of a release agent was 1: 100, and a die temperature was 230°C. The die used in a production process was a die-casting test bar die, and an obtained casting was labeled as A3.

### Example 4

The embodiment of the present invention provide a high-strength and high-toughness non-heat-treatable die-casting aluminum-silicon alloy, including the following components in percentage by weight:9.5% of Si, 0.25% of Mg, 0.6% of Mn, 0.15% of Ti, 0.15% of Cu, 0.02% of V, 0.05% of Er, 0.025% of Sr, 0.12% of Fe, 0.3% of other impurities and the balance of Al.

Preparation and die-casting processes for the high-strength and high-toughness non-heat-treatable die-casting aluminum-silicon alloy of the embodiment include the following steps:
1) drying: prepared raw materials: pure aluminum, pure Si, pure Mg, an Al-10Mn intermediate alloy, an Al-10Ti intermediate alloy, an Al-50Cu intermediate alloy, an Al-10Er intermediate alloy and an Al-5V intermediate alloy were pre-heated to 200°C for drying treatment; and
2) smelting: a furnace was heated to 755°C to melt the pure aluminum, then the Al-10Ti, Al-50Cu, Al-10Mn, Al-5V and pure Si alloys were added into the furnace, the furnace was cooled to 690°C after the intermediate alloys were melted, the pure Mg was pressed into a bottom area of a crucible by using a bell jar for melting, and then a melt was stirred for 5 min. Then the melt was heated to 720°C, nitrogen at a pressure of 0.4 MPa was introduced into the melt, a refining agent powder accounting for 0.4% of total weight of the melt was brought in, and nitrogen was introduced with a gas flow of 0.5 at 300r/min for 10 min to deslag and degas. Then the melt was left still for 12 min, and slagging-off treatment was completed; after refining was completed, the Al-10Er intermediate alloy was pressed into the bottom area of the crucible by using the bell jar for melting, and then the Al-10Er intermediate alloy was stirred for 5 min till the intermediate alloy was completely melted, and then the melt was left still for 12 min, and a blast furnace component analytical test was performed. High pressure casting was performed at 690°C after the test passed. An injections peed was 3 m/s, a casting pressure was 80 MPa, a ratio of a release agent was 1: 100, and a die temperature was 230°C. The die used in a production process was a die-casting test bar die, and an obtained casting was labeled as A4.

### Example 5

The embodiment of the present invention provide a high-strength and high-toughness non-heat-treatable die-casting aluminum-silicon alloy, including the following components in percentage by weight:9.5% of Si, 0.25% of Mg, 0.6% of Mn, 0.15% of Ti, 0.15% of Cu, 0.02% of V, 0.05% of La, 0.025% of Sr, 0.12% of Fe, 0.3% of other impurities and the balance of Al.

Preparation and die-casting processes for the high-strength and high-toughness non-heat-treatable die-casting aluminum-silicon alloy of the embodiment include the following steps:
1) drying: prepared raw materials: pure aluminum, pure Si, pure Mg, an Al-10Mn intermediate alloy, an Al-10Ti intermediate alloy, an Al-50Cu intermediate alloy, an Al-10La intermediate alloy and an Al-5V intermediate alloy were pre-heated to 200°C for drying treatment; and
2) smelting: a furnace was heated to 720°C to melt the pure aluminum, then the furnace was heated to 755°C and the Al-10Ti, Al-50Cu, Al-10Mn, Al-5V and pure Si alloys were added into the furnace, the furnace was cooled to 690°C after the intermediate alloys were melted, the pure Mg was pressed into a bottom area of a crucible by using a bell jar for melting, and then the pure Mg was stirred for 5 min. Then the melt was heated to 720°C, nitrogen at a pressure of 0.4 MPa was introduced into the melt, a refining agent powder accounting for 0.4% of total weight of the melt was brought in, and nitrogen was introduced with a gas flow of 0.5 at 300r/min for 10 min to deslag and degas. Then the melt was left still for 12 min, and slagging-off treatment was completed; after refining was completed, the Al-10La intermediate alloy was pressed into the bottom area of the crucible by using the bell jar for melting, and then the Al-10La intermediate alloy was stirred for 5 min till the intermediate alloy was completely melted, and then the melt was left still for 12 min, and a blast furnace component analytical test was performed. High pressure casting was performed at 690°C after the test passed. An injections peed was 3 m/s, a casting pressure was 80 MPa, a ratio of a release agent was 1: 100, and a die temperature was 230°C. The die used in a production process was a die-casting test bar die, and an obtained casting was labeled as A5.

### Example 6

The embodiment of the present invention provide a high-strength and high-toughness non-heat-treatable die-casting aluminum-silicon alloy, including the following components in percentage by weight:9.5% of Si, 0.25% of Mg, 0.6% of Mn, 0.15% of Ti, 0.15% of Cu, 0.02% of V, 0.05% of Ce, 0.025% of Sr, 0.12% of Fe, 0.3% of other impurities the balance of Al.

Preparation and die-casting processes for the high-strength and high-toughness non-heat-treatable die-casting aluminum-silicon alloy of the embodiment include the following steps:
1) drying: prepared raw materials: pure aluminum, pure Si, pure Mg, an Al-10Mn intermediate alloy, an Al-10Ti intermediate alloy, an Al-50Cu intermediate alloy, an Al-10Ce intermediate alloy and an Al-5V intermediate alloy were pre-heated to 200°C for drying treatment; and
2) smelting: a furnace was heated to 720°C to melt the pure aluminum, then the furnace was heated to 755°C and the Al-10Ti, Al-50Cu, Al-10Mn, Al-5V and pure Si alloys were added into the furnace, the furnace was cooled to 690°C after the intermediate alloys were melted, the pure Mg was pressed into a bottom area of a crucible by using a bell jar for melting, and then the pure Mg was stirred for 5 min. Then the melt was heated to 720°C, nitrogen at a pressure of 0.4 MPa was introduced into the melt, a refining agent powder accounting for 0.4% of total weight of the melt was brought in, and nitrogen was introduced with a gas flow of 0.5 at 300r/min for 10 min to deslag and degas. Then the melt was left still for 12 min, and slagging-off treatment was completed; after refining was completed, the Al-10Ce intermediate alloy was pressed into the bottom area of the crucible by using the bell jar for melting, and then the Al-10Ce intermediate alloy was stirred for 5 min till the intermediate alloy was completely melted, and then the melt was left still for 12 min, and a blast furnace component analytical test was performed. High pressure casting was performed at 690°C after the test passed. An injections peed was 3 m/s, a casting pressure was 80 MPa, a ratio of a release agent was 1: 100, and a die temperature was 230°C. The die used in a production process was a die-casting test bar die, and an obtained casting was labeled as A6.

### Example 7

The embodiment of the present invention provide a high-strength and high-toughness non-heat-treatable die-casting aluminum-silicon alloy, including the following components in percentage by weight: 10% of Si, 0.5% of Mg, 0.8% of Mn, 0.2% of Ti, 0.5% of Cu, 0.1% of V, 0.15% of La, 0.05% of Sr, 0.12% of Fe, 0.3% of other impurities the balance of Al.

Preparation and die-casting processes for the high-strength and high-toughness non-heat-treatable die-casting aluminum-silicon alloy of the embodiment include the following steps:
1) drying: prepared raw materials: pure aluminum, pure Si, pure Mg, an Al-10Mn intermediate alloy, an Al-10Ti intermediate alloy, an Al-50Cu intermediate alloy, an Al-10La intermediate alloy and an Al-5V intermediate alloy were pre-heated to 200°C for drying treatment; and
2) smelting: a furnace was heated to 755°C to melt the pure aluminum, then the Al-10Ti, Al-50Cu, Al-10Mn, Al-5V and pure Si alloys were added into the furnace, the furnace was cooled to 690°C after the intermediate alloys were melted, the pure Mg was pressed into a bottom area of a crucible by using a bell jar for melting, and then a melt was stirred for 5 min. Then the melt was heated to 720°C, nitrogen at a pressure of 0.4 MPa was introduced into the melt, a refining agent powder accounting for 0.4% of total weight of the melt was brought in, and nitrogen was introduced with a gas flow of 0.5 at 300r/min for 10 min to deslag and degas. Then the melt was left still for 12 min, and slagging-off treatment was completed; after refining was completed, the Al-10La intermediate alloy was pressed into the bottom area of the crucible by using the bell jar for melting, and then the intermediate alloy was stirred for 5 min till the intermediate alloy was completely melted, and then the melt was left still for 12 min, and a blast furnace component analytical test was performed. High pressure casting was performed at 690°C after the test passed. An injections peed was 3 m/s, a casting pressure was 80 MPa, a ratio of a release agent was 1: 100, and a die temperature was 230°C. The die used in a production process was a die-casting test bar die, and an obtained casting was labeled as A7.

### Example 8

The embodiment of the present invention provide a high-strength and high-toughness non-heat-treatable die-casting aluminum-silicon alloy, including the following components in percentage by weight: 8% of Si, 0.1% of Mg, 0.5% of Mn, 0.05% of Ti, 0.05% of Cu, 0.01% of V, 0.01% of La, 0.01% of Sr, 0.12% of Fe, 0.3% of other impurities the balance of Al.

Preparation and die-casting processes for the high-strength and high-toughness non-heat-treatable die-casting aluminum-silicon alloy of the embodiment include the following steps:
1) drying: prepared raw materials: pure aluminum, pure Si, pure Mg, an Al-10Mn intermediate alloy, an Al-10Ti intermediate alloy, an Al-50Cu intermediate alloy, an Al-10La intermediate alloy and an Al-5V intermediate alloy were pre-heated to 200°C for drying treatment; and
2) smelting: a furnace was heated to 755°C to melt the pure aluminum, then the Al-10Ti, Al-50Cu, Al-10Mn, Al-5V and pure Si alloys were added into the furnace, the furnace was cooled to 690°C after the intermediate alloys were melted, the pure Mg was pressed into a bottom area of a crucible by using a bell jar for melting, and then a melt was stirred for 5 min. Then the melt was heated to 720°C, nitrogen at a pressure of 0.4 MPa was introduced into the melt, a refining agent powder accounting for 0.4% of total weight of the melt was brought in, and nitrogen was introduced with a gas flow of 0.5 at 300r/min for 10 min to deslag and degas. Then the melt was left still for 12 min, and slagging-off treatment was completed; after refining was completed, the Al-10La intermediate alloy was pressed into the bottom area of the crucible by using the bell jar for melting, and then the intermediate alloy was stirred for 5 min till the intermediate alloy was completely melted, and then the melt was left still for 12 min, and a blast furnace component analytical test was performed. High pressure casting was performed at 690°C after the test passed. An injections peed was 3 m/s, a casting pressure was 80 MPa, a ratio of a release agent was 1: 100, and a die temperature was 230°C. The die used in a production process was a die-casting test bar die, and an obtained casting was labeled as A8.

### Comparative example 1

The comparative example of the present invention provide a high-strength and high-toughness non-heat-treatable die-casting aluminum-silicon alloy, including the following components in percentage by weight: 8.0% of Si, 0.25% of Mg, 0.6% of Mn, 0.15% of Ti,0.15% of Cu, 0.025% of Sr, 0.12% of Fe, 0.3% of other impurities and the balance of Al.

Preparation and die-casting processes for the high-strength and high-toughness non-heat-treatable die-casting aluminum-silicon alloy of the comparative example include the following steps:
1) drying: prepared raw materials: pure aluminum, pure Si, pure Mg, an Al-10Mn intermediate alloy, an Al-10Ti intermediate alloy and an Al-50Cu intermediate alloy were pre-heated to 200°C for drying treatment; and
2) smelting: a furnace was heated to 755°C to melt the pure aluminum, then the Al-10Ti, Al-50Cu, Al-10Mn and pure Si alloys were added into the furnace, the furnace was cooled to 690°C after the intermediate alloys were melted, the pure Mg was pressed into a bottom area of a crucible by using a bell jar for melting, and then a melt was stirred for 5 min. Then a melt was heated to 720°C, nitrogen at a pressure of 0.4 MPa was introduced into the melt, a refining agent powder accounting for 0.4% of total weight of the melt was brought in, and nitrogen was introduced with a gas flow of 0.5 at 300r/min for 10 min to deslag and degas. Then the melt was left still for 12 min, slagging-off treatment was completed, and a blast furnace component analytical test was performed. High pressure casting was performed at 690°C after the test passed. The die-casting process parameters and the die used for die casting were the same as those in the example 1, and the casting A9 was obtained.

### Comparative example 2

The comparative example of the present invention provide a high-strength and high-toughness non-heat-treatable die-casting aluminum-silicon alloy, including the following components in percentage by weight: 9.5% of Si, 0.25% of Mg, 0.6% of Mn, 0.15% of Ti, 0.15% of Cu, 0.025% of Sr, 0.12% of Fe, 0.3% of other impurities and the balance of Al.

Preparation and die-casting processes for the high-strength and high-toughness non-heat-treatable die-casting aluminum-silicon alloy of the comparative example include the following steps:
1) drying: prepared raw materials: pure aluminum, pure Si, pure Mg, an Al-10Mn intermediate alloy, an Al-10Ti intermediate alloy and an Al-50Cu intermediate alloy were pre-heated to 200°C for drying treatment; and
2) smelting: a furnace was heated to 755°C to melt the pure aluminum, then the Al-10Ti, Al-50Cu, Al-10Mn and pure Si alloys were added into the furnace, the furnace was cooled to 690°C after the intermediate alloys were melted, the pure Mg was pressed into a bottom area of a crucible by using a bell jar for melting, and then a melt was stirred for 5 min. Then the melt was heated to 720°C, nitrogen at a pressure of 0.4 MPa was introduced into the melt, a refining agent powder accounting for 0.4% of total weight of the melt was brought in, and nitrogen was introduced with a gas flow of 0.5 at 300r/min for 10 min to deslag and degas. Then the melt was left still for 12 min, slagging-off treatment was completed, and a blast furnace component analytical test was performed. High pressure casting was performed at 690°C after the test passed. The die-casting process parameters and the die used for die casting were the same as those in the example 1, and the casting A10 was obtained.

### Comparative example 3

The embodiment of the present invention provide a high-strength and high-toughness non-heat-treatable die-casting aluminum-silicon alloy, including the following components in percentage by weight:8.0% of Si, 0.25% of Mg, 0.6% of Mn, 0.15% of Ti,0.15% of Cu, 0.15% of V, 0.05% of La, 0.025% of Sr, 0.12% of Fe, 0.3% of other impurities and the balance of Al.

Preparation and die-casting processes for the high-strength and high-toughness non-heat-treatable die-casting aluminum-silicon alloy of the embodiment include the following steps:
1) drying: prepared raw materials: pure aluminum, pure Si, pure Mg, an Al-10Mn intermediate alloy, an Al-10Ti intermediate alloy, an Al-50Cu intermediate alloy, an Al-10La intermediate alloy and an Al-5V intermediate alloy were pre-heated to 200°C for drying treatment; and
2) smelting: a furnace was heated to 755°C to melt the pure aluminum, then the Al-10Ti, Al-50Cu, Al-10Mn, Al-5V and pure Si alloys were added into the furnace, the furnace was cooled to 690°C after the intermediate alloys were melted, the pure Mg was pressed into a bottom area of a crucible by using a bell jar for melting, and then a melt was stirred for 5 min. Then the melt was heated to 720°C, nitrogen at a pressure of 0.4 MPa was introduced into the melt, a refining agent powder accounting for 0.4% of total weight of the melt was brought in, and nitrogen was introduced with a gas flow of 0.5 at 300r/min for 10 min to deslag and degas. Then the melt was left still for 12 min, and slagging-off treatment was completed; after refining was completed, the Al-10La intermediate alloy was pressed into the bottom area of the crucible by using the bell jar for smelting, and then the Al-10La intermediate alloy was stirred for 5 min till the intermediate alloy was completely melted, and then the melt was left still for 12 min, and a blast furnace component analytical test was performed. High pressure casting was performed at 690°C after the test passed. The die-casting process parameters and the die used for die casting were the same as those in the example 1, and the casting A11 was obtained.

### Comparative example 4

The comparative example of the present invention provide a high-strength and high-toughness non-heat-treatable die-casting aluminum-silicon alloy, including the following components in percentage by weight:8.0% of Si, 0.25% of Mg, 0.6% of Mn, 0.15% of Ti,0.15% of Cu, 0.02% of V, 0.2% of La, 0.025% of Sr, 0.12% of Fe, 0.3% of other impurities and the balance of Al.

Preparation and die-casting processes for the high-strength and high-toughness non-heat-treatable die-casting aluminum-silicon alloy of the comparative example include the following steps:
1) drying: prepared raw materials: pure aluminum, pure Si, pure Mg, an Al-10Mn intermediate alloy, an Al-10Ti intermediate alloy, an Al-50Cu intermediate alloy, an Al-10La intermediate alloy and an Al-5V intermediate alloy were pre-heated to 200°C for drying treatment; and
2) smelting: a furnace was heated to 755°C to melt the pure aluminum, then the Al-10Ti, Al-50Cu, Al-10Mn, Al-5V and pure Si alloys were added into the furnace, the furnace was cooled to 690°C after the intermediate alloys were melted, the pure Mg was pressed into a bottom area of a crucible by using a bell jar for melting, and then a melt was stirred for 5 min. Then the melt was heated to 720°C, nitrogen at a pressure of 0.4 MPa was introduced into the melt, a refining agent powder accounting for 0.4% of total weight of the melt was brought in, and nitrogen was introduced with a gas flow of 0.5 at 300r/min for 10 min to deslag and degas. Then the melt was left still for 12 min, and slagging-off treatment was completed; after refining was completed, the Al-10La intermediate alloy was pressed into the bottom area of the crucible by using the bell jar for melting, and then the intermediate alloy was stirred for 5 min till the intermediate alloy was completely melted, and then the melt was left still for 12 min, and a blast furnace component analytical test was performed. High pressure casting was performed at 690°C after the test passed. The die-casting process parameters and the die used for die casting were the same as those in the example 1, and the casting A12 was obtained.

Mechanical properties of the castings A1-A12 prepared in the examples 1-8 and the comparative examples 1-4 are tested, and the test results are shown in Table 1.It can be found by comparing the mechanical properties of the castings A1, A2, A3 and A9 that by independently adding the element V or the rare earth element Er, the strength and ductility of the alloy are obviously improved, the tensile strength is increased by 27 MPa to the maximum extent, and the improved amplitude of the ductility reaches 24.1%. By adding the elements V and Er simultaneously, the plasticity of the alloy is more obviously improved, and the ductility of the casting is significantly increased from 8.7% (A9) to 14.9% (A3) with an increase amplitude of 71.2%. The above rule can also be found by comparing the mechanical properties of the castings A4 and A10. By means of compound addition of the elements V and Er, the plasticity of the die-casting aluminum alloy with high Si content (9.5 wt%) is significantly improved, so that the ductility is increased from 6.5 (the casting A10) to 12.9% (the casting A4), and the characteristics of high strength and high toughness of the alloy are satisfied. It is found by comparing the mechanical properties of the castings A4, A5, A6 and A10 that by means of compound addition of V and rare earth elements Er, La and Ce, the plasticity and tensile strength of the die-casting aluminum alloy can be significantly improved. The tensile strength of the castings A4-A6 is about 281 MPa, the ductility is about 12.8%, and compared with the casting A10, the tensile strength and the ductility are respectively increased by 16.5% and 97%. Thus, it is illustrated that the three RE rare earths included in the patent have significant effects to the alloy. It can be known by comparing the mechanical properties of the castings A5, A7, A8, A11 and A12 that within a range of composition of the alloy provided by the patent, by means of compound addition of V and rare earth elements, the yield strength of the die-casting aluminum alloy can be greater than 120 MPa, the tensile strength thereof can be greater than 260 MPa and the ductility thereof can be greater than 10% (the castings A5, A7 and A8), reflecting excellent mechanical properties of the alloy within the range of composition of the alloy provided by the patent. When V in the alloy reaches 0.15 (the casting A11) or the rare earth elements reach 0.2 (the casting A12), which exceeds the range of the patent, the ductility and the tensile strength of the alloy are significantly reduced, and particularly, the ductility of the alloy is reduced to be less than 8%, so that the high-strength and high-toughness die-casting aluminum alloy material cannot be obtained. In conclusion, in the range of composition of the alloy involved in the present invention, by adding the element V and RE elements (La, Er and Ce), the die-casting Al-Si alloy features high strength and high toughness in a non-heat treatment condition.

**Table 1 Tensile mechanical properties of castings A1-A12**

| Gro up | Major components | Yield strength/(MPa) | Tensile strength/(MPa) | Ductility/ % |
|---|---|---|---|---|
| A1 | Al8Si0.02V | 121 | 265 | 10.5 |
| A2 | Al8Si0.05Er | 125 | 279 | 10.8 |
| A3 | Al8Si0.02V0.05 Er | 129 | 281 | 14.9 |
| A4 | Al9.5Si0.02V0.0 5Er | 135 | 283 | 12.9 |
| A5 | Al9.5Si0.02V0.0 5La | 131 | 282 | 12.7 |
| A6 | Al9.5Si0.02V0.0 5Ce | 136 | 281 | 13.0 |
| A7 | Al10S10.1V0.15 La | 155 | 315 | 10.5 |
| A8 | Al8Si0.01V0.01 La | 123 | 267 | 13.2 |
| A9 | Al8Si | 121 | 252 | 8.7 |
| A1 0 | Al9.5Si | 136 | 241 | 6.5 |
| A1 1 | Al9.5Si0.15V0.0 5La | 134 | 251 | 7.9 |
| A1 2 | Al9.5Si0.02V0.2 La | 145 | 265 | 7.5 |

Microstructures of the castings A1-A12 respectively prepared in the above-mentioned examples 1-8 and comparative examples 1-4 are observed. The microstructures are shown in FIG. 1. It is found by comparing structures in A1(a), A2(b), A3(c) and A9(i) that with introduction of V and the rare earth element Er, the eutectic Si structure is obviously refined. When the alloy does not contain V and Er, the eutectic Si in the structure of the casting is of a layered structure in FIG. 1 (i), with a particle size of about 4 µm. With introduction of the element V or Er, the eutectic Si structure is transformed from being lamellar to being granular, and the particle size is significantly decreased to 1 µm, as shown in FIG. 1(a) and FIG. 1(b). By compound addition of V and Er, the size of the eutectic Si in the structure is further decreased, and the eutectic Si is a much smaller vermiform structure, as shown in FIG. 1 (c). Change of structural characteristics is closely related to change of mechanical properties. It is apparent that by introducing the elements V and Er, the eutectic Si structure can be significantly refined, and its shape is changed, so that the performance of the alloy changes significantly. It can be found by comparing structures of A4 and A10 that the compound action of the elements V and Er is also effective to the alloy structure with the high Si content. When the Si content is 9.5 wt.% and elements V and Er are not added into the alloy, the eutectic Si structure in the structure is in a thick broken line shape, and the maximum size of the fold line-shaped structure can reach up to 10 µm (as shown in FIG. 1 (j)).With introduction of the elements V and Er in the alloy, the eutectic Si structure in the alloy is significantly refined to be vermiform (as shown in FIG. 1 (d)), but there are block eutectic Si structures partially, which somewhat affects the plasticity of the alloy. Therefore, the plasticity of the alloy A3 is superior to that of the alloy A4.It is found by comparing the structures of the castings A4, A5, A6, A7, A8 and A10 that in the range of the alloy provided by the patent, by means of compound addition of the element V and the rare earth elements Er, La and Ce, the thick broken line-shaped structure in the die-casting aluminum alloy can disappear, so that the performance of the alloy is guaranteed. It can be known by comparing the structures of the castings A5, A11 and A12 that by adding excessive element V, second phases AIV can appear in the alloy structures, and by adding excessive rare earth elements, second phases AlLa can appear in the alloys. These second phases will reduce the plasticity of the alloys greatly. Generally, by introducing the compound action of the elements V and RE into the alloy provided by the patent, eutectic Si particles in the structures are finer and dispersive, and the shapes are greatly improved, so that the alloy has excellent mechanical properties due to the structural characteristic.

The above is merely embodiments of the present invention and does not hence limit the patent range of the present invention.

## Claims

1. A high-strength and high-toughness non-heat-treatable die-casting aluminum-silicon alloy, **characterized by** comprising the following components in percentage by weight: 8.0-10.0% of Si, 0.1-0.5% of Mg, 0.5-0.8% of Mn, 0.05-0.5% of Cu, 0.05-0.2% of Ti, 0.01-0.05% of Sr, 0.01-0.1% of V, 0.01-0.15% of RE, less than 0.2% of Fe, less than or equal to 0.4% of other impurities, and a balance of Al, wherein the RE is one or more of elements La, Ce, and Er.

2. A method for preparing the high-strength and high-toughness non-heat-treatable die-casting aluminum-silicon alloy according to claim 1, **characterized by** comprising the following steps:
S1: drying: pre-heating prepared raw materials of pure Al, pure Si, pure Mg, an Al-Mn intermediate alloy, an Al-Ti intermediate alloy, an Al-Cu intermediate alloy, an Al-RE intermediate alloy, and an Al-V intermediate alloy for a drying treatment; and
S2: smelting: adding the Al-Ti intermediate alloy, the Al-Cu intermediate alloy, the Al-Mn intermediate alloy, the Al-V intermediate alloy, and the pure Si after melting the pure Al by a preliminary heating to obtain a first resulting alloy melt, and performing a cooling on the first resulting alloy melt after melting the pure Si, the Al-Ti intermediate alloy, the Al-Cu intermediate alloy, the Al-Mn intermediate alloy, the Al-V intermediate alloy to obtain a second resulting alloy melt; pressing the pure Mg into a bottom of the second resulting alloy melt for melting to obtain a third resulting alloy melt, and performing a secondary heating on the third resulting alloy melt for a refinement of the third resulting alloy melt after completely melting the pure Mg to obtain a fourth resulting alloy melt; and then pressing the Al-RE intermediate alloy into a bottom of the fourth resulting alloy melt for melting to obtain a fifth resulting alloy melt, and leaving the fifth resulting alloy melt still after completely melting the fifth resulting alloy melt to obtain the high-strength and high-toughness non-heat-treatable die-casting aluminum-silicon alloy.

3. The method according to claim 2, **characterized in that** a pre-heating temperature in S1 is 190-210°C.

4. The method according to claim 2, **characterized in that** a preliminary heating temperature in S2 is 750-760°C.

5. The method according to claim 2, **characterized in that** a cooling temperature in S2 is 680-700°C.

6. The method according to claim 2, **characterized in that** a secondary heating temperature in S2 is 720-730°C.

7. The method according to claim 2, **characterized in that** the refinement in S2 specifically comprises: introducing a nitrogen with a refining agent powder into the third resulting alloy melt by using a rotary blowing device for an injection refining to obtain a first refined melt, performing a deslagging treatment and a degassing treatment on the first refined melt to obtain a second refined melt, then leaving the second refined melt still for 10-15 min, and completing a slagging-off treatment on the second refined melt to obtain the fourth resulting alloy melt.

8. The method according to claim 7, **characterized in that** process parameters for the rotary blowing device are as follows: a degassing revolution is 300-350 r/min; a degassing time is 5-10 min, a pressure of a gas source during the degassing treatment is 0.35±0.05 MPa, and a gas flow is 0.2-0.8 sccm.

9. The method according to claim 7, **characterized in that** the refining agent powder comprises one of magnesium chloride and calcium chloride.

## Patentansprüche

1. Hochfeste und hochzähe, nicht wärmebehandelbare Druckguss-Aluminium-Silizium-Legierung, **dadurch gekennzeichnet, dass** sie die folgenden Komponenten in Gewichtsprozent umfasst: 8,0-10,0% Si, 0,1-0,5% Mg, 0,5-0,8% Mn, 0,05-0,5% Cu, 0,05-0,2% Ti, 0,01-0,05% Sr, 0,01-0,1% V, 0,01-0,15% RE, weniger als 0,2% Fe, weniger als oder gleich 0,4% anderer Verunreinigungen und einen Restanteil an Al, wobei RE eins oder mehrere der Elemente La, Ce und Er ist.

2. Verfahren zur Herstellung der hochfesten und hochzähen, nicht wärmebehandelbaren Druckguss-Aluminium-Silizium-Legierung nach Anspruch 1, **dadurch gekennzeichnet, dass** es die folgenden Schritte umfasst:
S1: Trocknen: Vorwärmen vorbereiteter Rohstoffe aus reinem Al, reinem Si, reinem Mg, einer Al-Mn-Zwischenlegierung, einer Al-Ti-Zwischenlegierung, einer Al-Cu-Zwischenlegierung, einer Al-RE-Zwischenlegierung und einer Al-V-Zwischenlegierung für eine Trocknungsbehandlung und
S2: Schmelzen: Hinzufügen der Al-Ti-Zwischenlegierung, der Al-Cu-Zwischenlegierung, der Al-Mn-Zwischenlegierung, der Al-V-Zwischenlegierung und des reinen Si nach dem Schmelzen des reinen Al durch ein einleitendes Erwärmen, um eine erste resultierende Legierungsschmelze zu erhalten, und Durchführen einer Kühlung auf der ersten resultierenden Legierungsschmelze nach dem Schmelzen des reinen Si, der Al-Ti-Zwischenlegierung, der Al-Cu-Zwischenlegierung, der Al-Mn-Zwischenlegierung, der Al-V-Zwischenlegierung, um eine zweite resultierende Legierungsschmelze zu erhalten; Pressen des reinen Mg in einen Boden der zweiten resultierenden Legierungsschmelze zum Schmelzen, um eine dritte resultierende Legierungsschmelze zu erhalten, und Durchführen eines zusätzlichen Erwärmens auf der dritten resultierenden Legierungsschmelze für eine Raffination der dritten resultierenden Legierungsschmelze nach dem vollständigen Schmelzen des reinen Mg, um eine vierte resultierende Legierungsschmelze zu erhalten, und dann Pressen der Al-RE-Zwischenlegierung in einen Boden der vierten resultierenden Legierungsschmelze zum Schmelzen, um eine fünfte resultierende Legierungsschmelze zu erhalten, und Ruhenlassen der fünften resultierenden Legierungsschmelze nach dem vollständigen Schmelzen der fünften resultierenden Legierungsschmelze, um die hochfeste und hochzähe, nicht wärmebehandelbare Druckguss-Aluminium-Silizium-Legierung zu erhalten.

3. Verfahren nach Anspruch 2, **dadurch gekennzeichnet, dass** eine Vorwärmtemperatur in S1 190-210°C beträgt.

4. Verfahren nach Anspruch 2, **dadurch gekennzeichnet, dass** eine Temperatur des einleitenden Erwärmens in S2 750-760°C beträgt.

5. Verfahren nach Anspruch 2, **dadurch gekennzeichnet, dass** eine Kühltemperatur in S2 680-700°C beträgt.

6. Verfahren nach Anspruch 2, **dadurch gekennzeichnet, dass** eine Temperatur des zusätzlichen Erwärmens in S2 720-730°C beträgt.

7. Verfahren nach Anspruch 2, **dadurch gekennzeichnet, dass** die Raffination in S2 insbesondere Folgendes umfasst: Einführen eines Stickstoffs mit einem Raffinationsmittelpulver in die dritte resultierende Legierungsschmelze durch Verwendung einer rotierenden Blasvorrichtung für eine Injektionsraffination, um eine erste raffinierte Schmelze zu erhalten, Durchführen einer Entschlackungsbehandlung und einer Entgasungsbehandlung auf der ersten raffinierten Schmelze, um eine zweite raffinierte Schmelze zu erhalten, dann Ruhenlassen der zweiten raffinierten Schmelze für 10-15 min und Abschließen einer Abschlackungsbehandlung auf der zweiten raffinierten Schmelze, um die vierte resultierende Legierungsschmelze zu erhalten.

8. Verfahren nach Anspruch 7, **dadurch gekennzeichnet, dass** Prozessparameter für die rotierende Blasvorrichtung wie folgt sind: Eine Drehzahl bei der Entgasung beträgt 300-350 U/min; eine Entgasungszeit beträgt 5-10 min, ein Druck einer Gasquelle während der Entgasungsbehandlung beträgt 0,35 ± 0,05 MPa und ein Gasmengenstrom beträgt 0,2-0,8 sccm.

9. Verfahren nach Anspruch 7, **dadurch gekennzeichnet, dass** das Raffinationsmittelpulver entweder Magnesiumchlorid oder Calciumchlorid umfasst.

## Revendications

1. Alliage d'aluminium-silicium de coulée sous pression à haute résistance et haute ténacité non traitable thermiquement, **caractérisé en ce qu'**il comprend les composants suivants en pourcentage en poids : 8,0-10,0% de Si, 0,1-0,5% de Mg, 0,5-0,8% de Mn, 0,05-0,5% de Cu, 0,05-0,2% de Ti, 0,01-0,05% de Sr, 0,01-0,1% de V, 0,01-0,15% de RE, moins de 0,2% de Fe, moins de ou exactement 0,4% d'autres impuretés, et le reste étant de l'Al, dans lequel RE désigne un ou plusieurs éléments parmi La, Ce et Er.

2. Procédé de préparation de l'alliage aluminium-silicium de coulée sous pression à haute résistance et haute ténacité non traitable thermiquement selon la revendication 1, **caractérisé en ce qu'**il comprend les étapes suivantes :
S1 : séchage : préchauffer des matières premières préparées incluant de l'Al pur, du Si pur, du Mg pur, un alliage intermédiaire Al-Mn, un alliage intermédiaire Al-Ti, un alliage intermédiaire Al-Cu, un alliage intermédiaire Al-RE et un alliage intermédiaire Al-V pour un traitement de séchage ; et
S2 : fusion : ajouter l'alliage intermédiaire Al-Ti, l'alliage intermédiaire Al-Cu, l'alliage intermédiaire Al-Mn, l'alliage intermédiaire Al-V et du Si pur après fusion de l'Al pur par un chauffage préliminaire afin d'obtenir une première masse fondue d'alliage résultant, et effectuer un refroidissement sur la première masse fondue d'alliage résultant après fusion du Si pur, de l'alliage intermédiaire Al-Ti, de l'alliage intermédiaire Al-Cu, de l'alliage intermédiaire Al-Mn, de l'alliage intermédiaire Al-V afin d'obtenir une deuxième masse fondue d'alliage résultant ; presser du Mg pur au fond de la deuxième masse fondue d'alliage résultant pour fusion afin d'obtenir une troisième masse fondue d'alliage résultant, et effectuer un chauffage secondaire sur la troisième masse fondue d'alliage résultant pour un raffinage de la troisième masse fondue d'alliage résultant après fusion complète du Mg pur afin d'obtenir une quatrième masse fondue d'alliage résultant ; puis presser l'alliage intermédiaire Al-RE au fond de la quatrième masse fondue d'alliage résultant pour fusion afin d'obtenir une cinquième masse fondue d'alliage résultant, et laisser la cinquième masse fondue d'alliage résultant au calme après fusion complète de la cinquième masse fondue d'alliage résultant afin d'obtenir l'alliage d'aluminium-silicium de coulée sous pression à haute résistance et haute ténacité non traitable thermiquement.

3. Procédé selon la revendication 2, **caractérisé en ce qu'**une température de préchauffage en S1 est de 190-210°C.

4. Procédé selon la revendication 2, **caractérisé en ce qu'**une température de chauffage préliminaire en S2 est de 750-760°C.

5. Procédé selon la revendication 2, **caractérisé en ce qu'**une température de refroidissement en S2 est de 680-700°C.

6. Procédé selon la revendication 2, **caractérisé en ce qu'**une température de chauffage secondaire en S2 est de 720-730°C.

7. Procédé selon la revendication 2, **caractérisé en ce que** le raffinage en S2 comprend spécifiquement : introduire de l'azote avec une poudre d'agent de raffinage dans la troisième masse fondue d'alliage résultant en utilisant un dispositif de soufflage rotatif pour un raffinage par injection afin d'obtenir une première masse fondue raffinée, effectuer un traitement de décrassage et un traitement de dégazage sur la première masse fondue raffinée afin d'obtenir une deuxième masse fondue raffinée, puis laisser la deuxième masse fondue raffinée au calme pendant 10-15 min, et compléter un traitement de scorification sur la deuxième masse fondue raffinée afin d'obtenir la quatrième masse fondue d'alliage résultant.

8. Procédé selon la revendication 7, **caractérisé en ce que** les paramètres de procédé pour le dispositif de soufflage rotatif sont comme suit : une vitesse de rotation de dégazage est de 300-350 tour/min ; un temps de dégazage est de 5-10 min, une pression d'une source de gaz pendant le traitement de dégazage est de 0,35±0,05 MPa, et un flux de gaz est de 0,2-0,8 sccm.

9. Procédé selon la revendication 7, **caractérisé en ce que** la poudre d'agent de raffinage comprend l'un parmi le chlorure de magnésium et le chlorure de calcium.
